

Aug. 9, 1927.

1,638,541

C. E. McMANUS

CUSHION MATERIAL FOR BOTTLE CLOSURES

Filed July 6, 1922



Charles E. McManus, INVENTOR  
BY Frank P. Wentworth  
his ATTORNEY.

## UNITED STATES PATENT OFFICE.

CHARLES E. McMANUS, OF NEW YORK, N. Y.

## CUSHION MATERIAL FOR BOTTLE CLOSURES.

Application filed July 6, 1922. Serial No. 573,178.

My invention relates to cushion material for bottle closures, and more particularly to material adapted to be used in lieu of the natural, or composition, cork disks now 5 commonly used in closures of the type generally known as "Crown caps."

The main object of my invention is to provide cushion material embodying therein in a unitary structure in strip form, material 10 having sufficient resiliency to permit the formation of a tight seal when applied under pressure to the mouth of a bottle; sufficient rigidity to permit disks to be cut therefrom and applied to the metal shell of a closure 15 by a closure assembling machine, and a facing impermeable to gas and liquid, to be presented toward the contents of a bottle, said facing having sufficient flexibility or compressibility to yield with the cushioning 20 portion of the material as a closure containing same is applied to a bottle in the usual manner.

The cushion material embodying my invention, preferably consists of a plurality 25 of superimposed laminae firmly bonded together by means of suitable binders, adhesives or glues, one outer lamina being soft vulcanized rubber or rubber substitute, and the other outer lamina being of an oil or wax 30 fibrous material such as paper, an intermediate lamina preferably being provided for the purpose of giving additional body to the material and ensuring a better bonding of the rubber or rubber substitute lamina and 35 the oil or wax treated lamina with relation to each other in the strip material of which they form parts.

The invention consists primarily in cushion material for bottle closures embodying 40 therein, in a unitary structure and in strip form, a lamina of resilient material and a facing lamina permanently united thereto and consisting of a liquid and gas impervious 45 flexible fibrous material; and in such other novel characteristics as are hereinafter set forth and described and more particularly pointed out in the claims hereto appended.

In the accompanying drawing, I have 50 illustrated in perspective a short section of a strip of cushion material embodying my invention, broken away to disclose the different laminae.

In the embodiment of my invention shown 55 in the drawing, the cushion material is composed of one outer or cushion lamina *a* of soft vulcanized rubber or of a resilient rub-

ber substitute, and the other outer lamina or facing material *b* composed of suitable fibrous material, such as paper so treated with oil or wax as to be substantially impermeable by gas and liquid such as are ordinarily present in different beverages. Said cushion lamina *a* and said facing lamina *b* are united preferably by means of an intermediate lamina *c* of fibrous material, preferably untreated paper being used, since this lamina never contacts with the contents of a bottle and a better bond may be secured when this intermediate stratum is absorptive and permeable by the binder, adhesive 70 or glue used in uniting the cushion and facing laminae with relation to each other through said intermediate lamina.

The cushion lamina *a* may if desired be in the form of ordinary friction rubber applied to the lamina *c*, or may be bonded thereto by means of any suitable binder, adhesive or glue, as desired.

By reason of the impregnation of the lamina *b* with oil or wax and of the necessity 80 for securing flexibility in the binder, adhesive or glue used for uniting the lamina *b* to the intermediate lamina *c*, I preferably provide a stratum of a binder, adhesive or glue such as an asphaltum cement which has 85 the characteristic of being moisture repellent, between the laminae *b* and *c*, although any other flexible adhesive may be used in lieu thereof.

In the production of cushion material embodying my invention, the various laminae 90 are independently fed and collected, the adhesive being applied thereto during the feeding operation, said strips when collected, being forced together under pressure and 95 preferably in an elevated temperature so as to ensure a tight continuous joint between the adjacent laminae.

The finished strip as a whole, will possess the necessary thickness, resiliency and flexibility 100 to permit disks cut therefrom to be used instead of cork disks in bottle closures, and possesses the further advantage that it may be used in a machine in strip form and the cushion disks cut therefrom and applied 105 directly to the metal shell, each disk being free from surface voids of a magnitude which will not be closed as a result of the application of pressure to the closure in applying it to a bottle.

Ordinarily the thickness of the material 110 will be approximately one-half that of the

ordinary cushion disk, it being possible with this material to cup a disk when applying it to a shell and to fold or bend the edge of the disk upon itself so as to secure an edge 5 seal about the mouth of a bottle of greater thickness than the portion of the cushion with which the top of the mouth contacts. This thickened portion will of necessity have relatively greater resiliency than the portion 10 with which the top of a bottle contacts, so that a tight seal may be effected at the curvature at the top of the bottle as well as at the high point of the side of the bead. Furthermore, the cushion lamina *a* when a disk is 15 cupped and folded as described, will engage both the bead of a bottle and the material of the shell of the closure, which is a highly desirable condition in such closures.

In the production of closures embodying 20 the cushion material of my invention, the lamina *a* will be cemented to the shell of the closure, the arrangement of this lamina, however, being such that under no circumstances can moisture or gases from the bottle 25 penetrate through the adhesive securing the material to the shell, since the rubber or rubber substitute is immune to the action of water, and chemicals or gases ordinarily found in beverages, and furthermore when 30 cupped will vent such matter to atmosphere if it escapes through the seal.

It is not my intention to limit the invention to the exact adhesives or glues used, since there is a wide range of selection in 35 such materials as well as in the fibrous materials in the laminae *b* and *c*, nor to the method of producing the material.

I have found that the lamina *b* may be made of a special well known commercial 40 product consisting of an oil impregnated paper known in the art as insulating paper, which may be readily handled and bonded while possessing the desired non-absorptive and gas impervious properties.

45 Having described the invention, what I claim as new and desire to have protected by Letters Patent, is:—

50 1. Cushion material for bottle closures embodying therein, in a unitary structure and in strip form, a lamina of resilient ma-

terial, a facing lamina consisting of liquid and gas impervious fibrous material, an intermediate lamina of fibrous material bonded to said resilient material, and a stratum of moisture resisting cement bonding said intermediate and said facing lamina. 55

2. Cushion material for bottle closures embodying therein, in a unitary structure and in strip form, a lamina of soft vulcanized rubber, a facing lamina consisting of liquid and gas impervious fibrous material, an intermediate lamina of fibrous material bonded to said lamina of soft vulcanized rubber, and a stratum of moisture resisting cement bonding said intermediate and said 65 facing lamina.

3. Cushion material for bottle closures embodying therein in a unitary structure and in strip form, a lamina of resilient material, a facing lamina consisting of a liquid and gas impervious flexible fibrous material, and an intermediate lamina of absorptive, fibrous material readily permeable by a binding material, whereby the uniting of such other lamina is secured through the medium 75 of said intermediate lamina.

4. Cushion material for bottle closures embodying therein in a unitary structure and in strip form, a lamina of soft vulcanized rubber, a facing lamina consisting of a liquid and gas impervious flexible fibrous material, and an intermediate lamina of absorptive, fibrous material readily permeable by a binding material, whereby the uniting of such other lamina is secured through the 85 medium of said intermediate lamina.

5. Cushion material for bottle closures embodying therein in a unitary structure and in strip form, a lamina of soft vulcanized rubber, a facing lamina consisting of paper treated so as to be substantially impermeable 90 by gases and liquids, and an intermediate lamina of non-treated paper, bonded respectively to said rubber lamina and said treated paper lamina, whereby the uniting of said other lamina is secured through the medium 95 of said intermediate lamina.

In witness whereof I have hereunto affixed my signature, this 23rd day of June, 1922.

CHARLES E. McMANUS.